

Patented May 5, 1925.

1,536,653

# UNITED STATES PATENT OFFICE.

VERE B. BROWNE, OF BRACKENRIDGE, PENNSYLVANIA.

## METHOD OF MAKING SILICON STEEL.

No Drawing.

Application filed May 15, 1923. Serial No. 639,195.

To all whom it may concern:

Be it known that I, VERE B. BROWNE, a citizen of the United States, and a resident of Brackenridge, in the county of Allegheny and the State of Pennsylvania, have made a new and useful Invention in Methods of Making Silicon Steel, of which the following is a specification.

This invention relates to silicon steel and 10 a method of making the same.

An object of this invention is to provide a method by means of which ductile, homogeneous silicon steel of any desired silicon content free from inclusions and low in carbon may be readily made.

In building up certain laminated structures of electrical apparatus, silicon steel in the form of sheets is now commonly used. The presence of the silicon has a marked 20 influence on the magnetic and electrical qualities of the steel particularly in apparatus operating at high densities.

As the presence of silicon in the steel impairs its capacity for being rolled or otherwise worked, it is now common to add manganese to silicon steel to improve its workability. It is customary to make the manganese addition in the form of ferro-manganese or spiegeleisen but the addition of manganese in this manner necessarily increases 30 the carbon content of the finished steel to such an extent that its electrical properties are impaired.

A further object of this invention is to 35 provide a method of making iron silicon manganese alloys having a carbon content sufficiently low as not to impair its value for use in electrical apparatus requiring high magnetic permeability and low hysteresis.

40 In making silicon steel, the preferred method of obtaining the necessary silicon content is to place the desired amount of ferro-silicon which has first been raised to red heat, in the ladle and to add to this, the molten steel.

The method by which I attain the objects of this invention consists in reducing manganese from manganese ore in the ladle in the presence of the ferro-silicon. The 45 amount of manganese ore (manganese oxide) must be in excess of the theoretical amount necessary to give the desired manganese content to the finished steel. It is preferable, but not necessary, to mix a small 50 amount of fluorspar with the manganese ore before the same is added to the ladle. Since

the reaction of reduction will not be complete, there will remain in the ladle a small quantity of free manganese oxide which will combine with the silica present forming a 60 silicate of manganese. Silicate of manganese has a relatively low fusing point and in the presence of the fluorspar forms a solvent for any refractory material entrapped in the steel.

65 The amount of manganese ore added in the ladle will depend upon the percentage of manganese desired in the finished steel and the quality of the ore used, but it must always be in excess of the theoretical 70 amount in order to obtain the desired manganese content in the finished steel. I find that it is preferable to place the ferro-silicon in the ladle after the same is brought to a red heat and to place the manganese 75 ore in the ladle before the molten steel is tapped into the same. When the manganese ore is added at this time, the silicon present combines with the oxygen in the manganese ore to form silica and manganese metal is precipitated and alloys with the steel.

80 As this reaction is not complete under such conditions, there is always an excess of manganese oxide remaining in the ladle. This serves as a cleanser by combining with any refractory materials present such as silica and alumina. The silicates of manganese and double silicate of alumina and manganese have, comparatively speaking, 85 low fusing points and on this account readily float to the surface of the ladle absorbing and taking with them any excess of silica and alumina which may be entrapped in the molten steel.

90 These silicates are thus eliminated by direct combination and by mechanical absorption and separation.

Having thus described my invention, 100 what I claim is:—

1. The method of adding manganese to steel, which consists in directly reducing manganese from manganese ore by bringing together in the ladle manganese ore and molten steel.

105 2. The method, which consists in directly reducing manganese from manganese ore by bringing together in the ladle manganese ore and molten steel, whereby manganese is added to the steel, and refractory impurities such as alumina and silica are removed by combining with manganese ox-

ide to form silicates of manganese and aluminum having relatively low fusing temperatures and are eliminated by direct combination and by mechanical absorption and separation.

3. The method of making an iron silicon manganese alloy which consists in directly reducing manganese from manganese ore in the ladle in the presence of molten steel and ferro-silicon.

4. The method of making an iron silicon manganese alloy low in carbon which consists in mixing ferro-silicon and manganese oxide with molten steel in the ladle before teeming.

In testimony whereof, I have hereunto subscribed my name this 8th day of May, 1923.

VERE B. BROWNE.